

## UNITED STATES PATENT OFFICE

2,070,679

PROCESS FOR PREPARING NONMETALLIC  
ARTICLES FOR ELECTRO-PLATINGRudolf Peböck and Kurt Bergstein, Berlin,  
GermanyNo Drawing. Application August 4, 1934, Serial  
No. 738,546. In Germany August 7, 1933

2 Claims. (Cl. 204—8)

The invention relates to a process for preparing for electro-plating solid non-metallic bodies, especially those made of compressed materials, such as artificial resin and similar substances, by preliminary coppering in the cold.

It has been proposed to prepare in the cold non-metallic articles to be electro-plated by first applying to the article by means of a resin varnish a layer of metal which is electrically conductive and then immersing the article so treated in a non-galvanic copper bath (coppering by immersion), the actual electro-deposition (such as nickelizing, silvering etc.) following.

This process has the disadvantage that the article rendered conductive by the layer of metal powder receives in the non-galvanic copper bath an extremely thin coat of copper which does not adhere to the base substance and which will not withstand the mechanical stresses imposed by polishing or grinding while at the same time this coating of copper does not form an effective base for the subsequent treatment in alkali baths.

It has furthermore been proposed to produce non-metallic articles suitable for the actual electro-deposition treatment by rendering them electrically conductive by means of a solution of copper bronze and celluloid lacquer, and then immersing the articles into a galvanic acid copper bath. It has been found, however, that the adhesiveness of the coatings so produced is not perfect and particularly that it is not possible to polish these coatings without the coating dissolving, at least in part.

These disadvantages are avoided according to the invention by effecting the preliminary coppering in the following manner.

An electrically conductive layer of metal powder which has a lower potential than copper is applied to a non-metallic article by means of a suitable varnish such as a copal or other resin varnish, the surface of the article being roughened or similarly treated in known manner. The article so treated is immersed in an acid copper, bath which acts as a binding bath without the use of an electric current acting from without, in order to coat it with a closely adhering thin copper skin which ensures a uniform distribution of the current in a subsequent electro-deposition operation for the formation of a second film of copper. This galvanic coppering proceeds in the usual

manner, that is to say the article leaving the binding bath is placed in a galvanic acid copper bath in the manner usual in the manufacture of electrotype plates. Following this electrotype coppering operation, which advantageously lasts for from one to two hours and by means of which a base, which can be mechanically treated, is applied to the article, there is carried out the usual improving operation, namely nickelizing, silvering, etc.

In order to be certain that the copper skin completely covers the electrically conductive article it is advantageous to select as the electrically conductive layer a metallic powder the colour of which differs sufficiently from the colour of the copper such for example as an alloy of lead and zinc.

We claim:

1. The process for preparing moulded articles of artificial resin for electro-plating which consists in roughening the external surfaces of the articles, applying to the roughened surfaces by means of a varnish a thin electrically conductive layer of a metal alloy powder containing lead and a metal of a potential lower than copper and of a color differing from that of copper, immersing the articles in a first acid copper bath, removing them from said first acid copper bath after the formation of a thin copper skin on their surfaces, placing them in a second acid copper bath, and applying an electric current for electrolytic deposition of a copper layer on the copper skin formed in the first acid copper bath.

2. The process for preparing non-metallic articles for electro-plating which consists in roughening the external surfaces of the articles, applying to the roughened surfaces by means of a varnish a thin electrically conductive layer of a metal alloy powder containing lead and a metal of a potential lower than copper and of a color differing from that of copper, immersing the articles in a first acid copper bath, removing them from said first acid copper bath after the formation of a thin copper skin on their surfaces, placing them in a second acid copper bath, and applying an electric current for electrolytic deposition of a copper layer on the copper skin formed in the first acid copper bath.

RUDOLF PEBÖCK.  
KURT BERGSTEIN. 50